

# United States Patent [19]

Douglas

[11] Patent Number: 4,798,077

[45] Date of Patent: Jan. 17, 1989

[54] METHOD FOR PRODUCING A FAMILY OF FORGED RING ROLLING PREFORMS AND FORGING DIE THEREFOR

4,050,283 9/1977 Schober ..... 72/360  
4,084,419 4/1978 Dittrich et al. ..... 72/68  
4,590,782 5/1986 Leykamm et al. ..... 72/354

[75] Inventor: James R. Douglas, Mentor, Ohio

OTHER PUBLICATIONS

[73] Assignee: Eaton Corporation, Cleveland, Ohio

SAE paper number 841085.

[21] Appl. No.: 14,428

Metals Handbook, Thomas, 8th edition, vol. 5.  
Thyssen Industrie AG Position 84/85, pp. 26-27.

[22] Filed: Feb. 12, 1987

Primary Examiner—W. Donald Bray

Attorney, Agent, or Firm—H. D. Gordon

[51] Int. Cl.<sup>4</sup> ..... B21J 1/06; B21D 22/00

## [57] ABSTRACT

[52] U.S. Cl. ..... 72/360; 29/159.2;  
72/331; 72/354; 72/68

A method (FIGS. 4 and 4a) for making ring rolling preforms (102) of substantially toroidal shape for ring rolling (84) into substantially rectangular cross-sectional wall shaped forging blank rings (104) to be precision forged (86) into near net ring gear forgings (106) for heavy-duty drive axle ring gears (14) is provided. The method, and the preform forging die (138) used therefor, allow a series of preforms having between eighty percent (80%) to one hundred percent (100%) of the volume of the toroidal cavity portion (150) of the preform die to be forged utilizing a common die.

[58] Field of Search ..... 72/352, 359, 360, 331,  
72/70, 111; 29/159.2, 420.5

13 Claims, 10 Drawing Sheets

## [56] References Cited

### U.S. PATENT DOCUMENTS

- |           |         |                       |        |
|-----------|---------|-----------------------|--------|
| 1,205,301 | 11/1916 | Williams              | 72/360 |
| 1,971,027 | 8/1934  | Bell                  | .      |
| 1,991,486 | 2/1935  | Bell                  | .      |
| 2,058,007 | 10/1936 | Edelmeier             | 72/331 |
| 3,298,219 | 1/1967  | Schober               | .      |
| 3,382,693 | 5/1968  | Rozhdestvensky et al. | .      |
| 3,832,763 | 9/1974  | Schober               | 72/360 |
| 4,015,461 | 4/1977  | Schober               | 72/360 |



FIG. 1

PRIOR ART



FIG. 2A



FIG. 2B







FIG. 4







FIG. 6



**METHOD FOR PRODUCING A FAMILY OF FORGED RING ROLLING PREFORMS AND FORGING DIE THEREFOR**

**BACKGROUND OF THE INVENTION**

**1. Related Applications**

This application is related to Ser. No. 014,426 and Ser. No. 014,429, both filed Feb. 12, 1987.

**2. Field of the Invention**

This invention relates to a method for producing near net forgings for ring gears, especially ring gears of the hypoid, straight-bevel or spiral-bevel type for heavy-duty trucks drive axles, from rolled ring shaped blanks produced by ring rolling of forged preforms. In particular, the present invention relates to a method for producing a family of different volume forged ring rolling preforms utilizing a common preform forging die and to the preform forging die therefor.

**3. Description of the Prior Art**

Right angle drive trains for heavy-duty drive axles utilizing pinion gears/ring gear gear-sets are well known in the prior art, as may be seen by reference to U.S. Pat. Nos. 3,265,173; 4,018,097; 4,046,210; 4,050,534 and 4,263,334, by reference to allowed U.S. patent application Ser. No. 761,262, filed Aug. 1, 1985, and assigned to the Assignee of this invention, and to SAE Paper No. 841085, the disclosures of all of which are hereby incorporated by reference. Such gear-sets are usually of the well known spiral-bevel or hypoid gear type or some modification or derivative thereof.

Forging processes for the production of gear forgings/gear blanks having at least partially formed teeth are well known in the prior art, especially for relatively smaller sized bevel gears, such as differential pinion and side gears, as may be seen by reference to U.S. Pat. Nos. 3,832,763; 4,050,283 and 4,590,782, the disclosures of which are all hereby incorporated by reference.

The ring rolling process whereby generally annular rings are ring rolled from ring rolling preforms is also well known in the prior arts as may be seen by reference to U.S. Pat. Nos. 1,971,027; 1,991,486; 3,230,370; 3,382,693; and 4,084,419, and to Metals Handbook, 8th Edition, Volume 5, American Society for Metals, Pages 106 to 107, "Ring Rolling", the disclosures of all of which are hereby incorporated by reference.

In the past, due to the relatively massive size, ring gears for heavy-duty trucks have been produced by a method comprising the forging of a gear blank having outer diameter flash and a center slug, trimming of the forged gear blank, a normalizing heat treatment of the trimmed gear blank, extensive machining of the gear blank to rough and then final cut gear teeth therein, other machining of surfaces and mounting bores, a carburizing heat treatment, a lapping operation wherein the ring gear and a pinion gear are rotated in meshing engagement in a lapping compound, and then maintaining the ring gear and pinion gear as a matched set to be used only in connection with one another.

While the prior art method for producing ring gears for heavy-duty trucks has been utilized for many years as have the ring gears and ring gear/pinion gear-sets produced thereby, this method is not totally satisfactory as the billets used therein are of a considerably greater volume than the finished ring gear representing undesirably high material and heating costs, cutting of the gear teeth from the gear blanks is an expensive and time consuming operation and teeth formed by a cutting

process do not possess the desirable grain flow characteristics inherent in gear teeth formed by a material deformation process and thus do not provide the performance of formed gear teeth. Also, as the lapped ring gear/pinion gear gear-sets are only usable as a matched pair, great care must be taken to maintain the gear-sets in matched pairs and damage to either the ring gear or pinion gear will render the entire gear set useless.

The forging of hollow members from rolled rings to save material is generally known in the prior art. However, this process usually is economical only for high volume production because ring rolling of the blanks requires a forming operation (on a forge press or hammer) to produce the annular preform to be ring rolled. The material savings, and other savings associated therewith, were not sufficient to make such a method economically desirable, especially as to the relatively larger more costly ring gears, in the volume and variety of sizes and ratios associated with heavy-duty drive axles (i.e. drive axles utilized with heavy-duty trucks, off-the-road construction vehicles and the like). This was because prior art production of preforms, as with most other forging operations, had the conventional wisdom that the preform die must be filled to nearly one hundred percent (100%) of its theoretical capacity and thus each different sized preform would require a separate die and, for relatively small lots, the material savings would be more than offset by the additional preform tooling and press setups normally required.

**SUMMARY OF THE INVENTION**

In accordance with the present invention, the drawbacks of the prior art are overcome, or minimized, by the provision of a method for the production of drive axle ring gears for heavy-duty vehicles which is economical feasible in view of the relatively large size relatively low volume and relatively large variety of sizes and ratios associated with such heavy-duty drive axles. The method allows for considerable material and energy savings in view of the prior art methods, and eliminates the necessity for lapping of the ring gear with a mating pinion gear to produce a matched ring gear/pinion gear gear set and thereafter utilizing said ring gear only as a matched component to the pinion gear lapped therewith. Further, relative to the production of forged preforms to be ring rolled into rolled ring forging blanks, the necessity for providing an individual preform forging die for each different preform is eliminated.

The above is accomplished by the forging of a near net ring gear forging from a rolled ring forging blank produced by the ring rolling method and of very carefully controlled volume. The rolled ring blank is produced on a ring rolling machine from a forged ring rolling preform of carefully controlled volume and of a generally toroidal shape which is forged in a preform forging die suitable for the forging of a family of preforms having a common height, a common interior diameter and a volume in the range of eighty to one hundred percent (80% to 100%) of the largest preform member of the family. Accordingly, a common or universal preform die may be utilized to forge a large variety of ring rolling preforms and the expense related to preform tooling and preform press set-up time is minimized.

Accordingly, it is an object of the present invention to provide a new and improved method for the production of heavy-duty drive axle ring gears.

A further object of the present invention is to provide an improved method for the production of forged ring rolling preforms, and an improved forging die therefor, allowing a family, or grouping, of different sized preforms to be produced on a common forging die.

This and other objects and advantages of the present invention will become apparent from a reading of the detailed description of the preferred embodiment taken in view of the drawings.

#### BRIEF DESCRIPTION OF THE DRAWINGS

FIG. 1 is a partial sectional view of a typical prior art 15 heavy-duty drive axle of the type utilizing rear gear/pinion gear drive gears.

FIGS. 2A and 2B, respectively, illustrate prior art 20 spiral bevel and hypoid, respectively, ring gear/pinion gear drive gears.

FIGS. 3 and 3A, respectively, are schematic block 25 diagrams of the metal deformation and post metal deformation portions, respectively, of the prior art method for producing ring gears for heavy-duty vehicle drive axles.

FIGS. 4 and 4A, respectively, are schematic block 30 diagrams of the metal deformation and post metal deformation portions, respectively, of the method of the present invention for producing ring gears for heavy-duty vehicle drive axles.

FIG. 5 is a schematic block diagram illustration of the 35 ring rolling preform production portion of the method illustrated in FIGS. 4 and 4A.

FIG. 6 is a schematic cross-sectional view of the 40 forging die utilized in the method of the present invention to produce forged ring rolling preforms.

FIGS. 7 and 8, respectively, are enlarged cross-sectional schematic views of the forging die illustrated in FIG. 6, illustrating forging of preforms having approximately one hundred percent (100%) and eighty five 45 percent (85%), respectively, of the theoretical volume of the preform forging die cavity.

FIG. 9 is a schematic illustration of the ring rolling process portion of the method illustrated in FIGS. 4 and 4A.

FIG. 10 is a cross-sectional view of the near net gear 50 forging produced by the method illustrated in FIG. 4.

#### DESCRIPTION OF THE PREFERRED EMBODIMENT

In the following description of the present invention, certain terms will be utilized for purposes of reference only and are not intended to be limiting. The terms "upward", "downward", "rightward" and "leftward" refer to directions in the drawings to which reference is made. The terms "inward" and "outward", respectively, refer to directions toward and away from, respectively, the geometric center of the device described. Said terminology will include the words above specifically mentioned, derivatives thereof and words 55 of similar import.

The method, and the forging die therefor, of the present invention involves a portion of a process for producing ring gears for heavy-duty vehicle drive axles. An essential feature of the process for producing such ring gears involves the precision forging of near net ring gear forging from a low to medium carbon level carbon and alloy steel (usually having a carbon

content of 0.05% to 0.5% weight) such as AISI 8620A, 8622A, 8625A, 8822A, 4817H and 9310A. The term "AISI" refers to the American Iron Steel Institute and the steel classification standards established thereby. However, the process of the present invention is not limited to any particular specific type of low to medium carbon level carbon and alloy steel.

As used herein, the term "precision forging" and derivatives thereof, will refer to a forging process (i.e. bulk deformation of a workpiece under pressure) capable of producing "net parts", i.e. part is usable as forged (subject to heat treating and other non-machining steps) or "near net parts", i.e. forging usually requiring 0.030 inch or less of material removal from any functional surface.

The use of ring gear/pinion gear right angle gear-sets in the drive train of heavy-duty drive axles is well known in the prior art. Referring to FIG. 1, a single reduction drive axle 10 utilizing such a gear-set 11 comprising a pinion gear 12 meshingly engaged with a ring gear 14 is illustrated. A differential assembly 16 is fixed to the ring gear by bolts 17 for driving the two axle shafts 18 and 20. The axis of rotation 22 of the pinion gear 12 is substantially perpendicular to the axis of rotation 24 of ring gear 14 (and of differential assembly 16 and drive axles 18 and 20). Heavy-duty drive axles of this, and of the two-speed and the planetary double reduction type, are well known in the prior art and may be appreciated in greater detail by reference to above-mentioned U.S. Pat. Nos. 4,018,097 and 4,263,824 and allowed U.S. patent application Ser. No. 761,262, filed Aug. 1, 1985 and assigned to the Assignee of this invention.

Most heavy-duty drive axles utilize right angle ring gear/pinion gear drive-sets of either the spiral bevel or hypoid type as illustrated in FIGS. 2A and 2B, respectively. The method of the present invention, and the forging die therefor, is intended for the production of spiral bevel and hypoid gearing and/or derivatives or modifications thereof. As may be seen, in a spiral bevel gear-set, FIG. 2A, the axes of rotation 22 and 24 are perpendicular and intersect while in a hypoid gear-set, FIG. 2B, the axes 22 and 24 are offset by a distance 26. The hypoid offset is usually about 1.00 to 2.00 inches, in a gear set having a twelve to eighteen inch pitch diameter ring gear. The ring gears 14 are provided with a mounting bore 28 for receipt to the differential assembly 16 and drive shafts 18 and 20, and a plurality of bolt circle bores 30 for receipt of the bolt and nut assemblies 17 for mounting of the ring gear to the differential assembly 16.

As is known, spiral bevel gears provide, in theory, a totally rolling, not sliding, gear contact at the pitch line whereas hypoid gear-sets can be smaller, but do have a greater degree of sliding gear contact at the pitch line. In recent years, with improvements in gear design and lubrication, sliding contact is not the major problem it once was and hypoid gear-sets for heavy-duty drive axles have become more accepted. The present invention will, for ease of explanation only, be illustrated in connection with a spiral bevel gear-set, it being understood that the present invention is equally well suited for both spiral bevel and hypoid gear-sets as well as modifications thereof. The features and advantages of spiral bevel and hypoid ring gear/pinion gear gear-sets are well known in the prior art as may be seen by reference to above-mentioned SAE Paper No. 841085.

The most significant steps of the prior art process for producing heavy-duty vehicle drive axle ring gears 14 is schematically illustrated in block diagram form in FIGS. 3 and 3A. Briefly, the portion of the prior art process illustrated in FIG. 3 is that portion performed on the initial heated billet and comprises primarily deformation and trimming operations while that portion schematically illustrated in FIG. 3A illustrates the operations performed post metal deformation on the trimmed gear blank 34. It is noted that for both the prior art process illustrated in FIGS. 3 and 3A and the process of the present invention as illustrated in FIGS. 4 and 4A, the final ring gear 14 to be produced is comparable and has a weight of approximately 49.75 pounds.

The metal deformation portion of the prior art process includes the following sequential steps described in greater detail below: billet preparation and heating 36, upsetting or busting 38, blocking 40, forging of the gear blank 42, and trimming of the gear blank 44.

For purposes of description and comparison, the ring gear 14 to be produced by both the prior art method and the method of the present invention will be a single speed ring gear having an outer diameter of approximately sixteen and one-half (16 $\frac{1}{2}$ ) inches and net weight of approximately 49.75 pounds and substantially identical specifications. The billet or slug 32 is cut out to a predetermined size and shape from bar stock or suitable gear material, namely a low to medium carbon level carbon or alloy steel. The billet 32 is then heated to a pre-selected appropriate forging temperature (normally about 2250°-2350° F.). To minimize scaling (oxidation) and depth of scaling of the heated billet, the billet is preferably heated as quickly as practical.

In the upsetting and blocking steps, 38 and 40, respectively, the heated workpiece is first upset to form a generally pancake shaped billet 46 to remove scale and is then blocked to form a forging preform 48. Steps 38 and 40 require separate blows of a press and, due to the relatively massive size of the workpiece, are not performed simultaneously. In the gear blank forging step 42, the forging preform 48 is forged into an untrimmed gear blank 50. It is noted that untrimmed gear blank 50 comprises a relatively large center slug portion 52 and a relatively large exterior flash portion 54 which is formed at the parting lines of the forging die as is well known in the art. In the trimming step 44 the center slug portion 52 and exterior flash 54 is trimmed from the gear blank to provide a trimmed gear blank 56. Gear blank 56 is not provided with any partially formed teeth.

While the desirability of forming forged gear blanks similar to 56 with at least partially formed gear teeth therein has been well known in the prior art, it has not been economically feasible by the conventional forging method illustrated in FIG. 3 due to the relatively massive size of the heavy-duty drive axle ring gears involved. The reason for this is the number of steps which would be involved, namely upsetting or busting, blocking to form a preform, finish forging, trimming and then the forging of teeth would involve such a large number of steps that the workpiece would lose too much of its heat (i.e. would become too cool), for proper forging of the teeth. This is especially true in view of the relatively larger surface areas of the workpiece in contact with the tooling as is well known in the prior art. Additionally, if teeth were formed after the busting and blocking steps, scale produced in these steps would result in unacceptable surface quality. Additionally, if an attempt

was made to forge teeth into workpiece 56 in its relatively cool condition, the relatively large size of the required press and the relatively large pressures required for forging teeth at the relatively depressed temperature of the workpiece would quickly destroy tooling rendering the process further economically infeasible.

The remainder or post metal deformation system of the prior art process is schematically illustrated in FIG. 10 3A and includes the following sequential steps described in greater detail below; normalizing heat treatment 58, a surface turning operation 60, drilling of the bolt circle bores 62, rough cutting of the gear teeth 64, finish cutting of the gear teeth 66, a carburizing heat 15 treatment of the work piece 68, a finished machining operation 70, a lapping operation with a mated pinion 72 and a matched ring gear/pinion gear-set marking and gear-set maintenance procedure 74.

The trimmed gear blank, or workpiece, 56 is then 20 subjected to a normalizing heat treatment to optimize metallurgical structure thereof in preparation for machining. A normalizing heat treatment of forged gear steels of the type involved typically comprises a heating, soaking and/or controlled cooling operation. After 25 the normalizing heat treatment, all of the surfaces of the normalized gear blank are subject to a turning operation to provide proper surfaces for later locating and machining. In step 62, the bolt circle bores 30 are drilled into the mounting flange 76.

It is noted that throughout the description of the prior 30 art method and the description of the method of the present invention that, for purposes of ease of description, portions of unfinished workpieces will be referred to by the same name and reference numeral as portions of the finished ring gear 14. By way of example, the center aperture of the trimmed gear blank 56 will be referred to as the mounting bore 28 although further machining is required until this central bore is of the exact dimensions of the mounting bore on the finished ring gear 14.

In operations 64, 66, respectively, teeth are cut into the workpiece in a rough cut and then finished cut procedure, respectively. The cutting of spiral bevel, hypoid and/or modified gear teeth is a well known 45 procedure, and may be performed by gear cutting machinery sold by Gleason Works under the tradename "Gleason Generator" or by the Oerlikom Company and sold under the tradename of "Spiromatic". After the gear cutting operations, the workpieces are subjected to 50 a carburizing heat treatment in step 68. As is known, a carburizing heat treatment involves a heating of the workpieces (usually to 1600°-1700° F.) in a high carbon atmosphere to cause a diffusion of carbon into the surfaces to harden the surfaces and provide hard, high carbon surfaces for improved wear of the finished product. After the carburizing heat treatment, the hardened workpiece is subject to a finish machining of the bolt circle and mounting bores, 28 and 30.

As the generated or cut gear tooth surfaces have been 60 subject to a heat treatment after cutting of the tooth surfaces, even in a carefully controlled heat treatment process some distortion will result. Accordingly, to provide acceptable performance of the ring gear/pinion gear gear-sets, i.e. to provide the necessary surface 65 quality, it is necessary that a carburized ring gear and pinion gear be subject to the lapping operation of step 72. In the lapping process, a matched set of ring gear and pinion gear are meshingly engaged and then rotated

under a simulated load while a lapping compound is sprayed into the gear tooth mesh. Typically, the rotational axis 22 of the pinion gear is pivoted relative to the rotational axis 24 of the ring gear so that the proper surface treatment is provided to the entire tooth surfaces of both the ring gear and pinion. The lapping compound is a relatively fine abrasive suspended in a lubricant. Once lapped together, the lapped ring gear and pinion gear are a matched set, are only satisfactorily usable as a matched set and are only properly used or replaced as a pair. Accordingly, it is necessary that the matched set be marked as such and that great care be maintained to maintain the set. Usually, this requires special pallets and containers for gear makers, axle assemblers and also at the location of servicing. The requirements for maintaining and utilizing the ring gear/pinion gear gear-sets only as a matched pair does, of course, involve additional expense. This is especially true for those types of gear-set designs wherein a common ring gear may be utilized with pinion gears having differing numbers of teeth as is disclosed in allowed U.S. patent application Ser. No. 761,262, filed Aug. 1, 1985 and assigned to the Assignee of the present invention.

FIGS. 4 and 4A, respectively, illustrate the most significant steps of the metal deformation and post metal deformation portions, respectively, of the present invention for producing ring gears for heavy-duty vehicle drive axles. The process includes the following sequential steps, each of which will be described in greater detail below; preparation and heating of the billet 80, forging of a ring rolling preform 82, ring rolling a rolled ring forging blank 84, precision forging of a near net gear forging 86, a normalizing heat treatment which will not be required for many of the alloys expected to be used in connection with the present invention 88, a semi-finish machining operation 90, a carburizing heat treatment 92, a finished machining for the center and mounting bores 94 and a finish grinding of the final gear teeth profiles 96. As will be discussed in greater detail below, it is important to note that the finish grinding 96 of the final gear tooth profiles occurs after the final heat treatment 92 of the gear (and pinion) and thus the tooth profiles will not be subject to distortion in a subsequent heat treatment. If the pinion gears 12 are manufactured by a similar process, the necessity for a later lapping operation and for the necessity for utilizing the ring gears only in connection with a matched pinion is eliminated.

A billet or slug 100 is cut to a carefully controlled predetermined size and shape from bar stock of a carburizing grade of low to medium carbon level carbon and alloy steel which has been cleaned. Contrary to prior art practice of requiring cleaning by grinding, usually a centerless grinding or the like, of billets to be utilized of near net forgings, the present practice does not require cleaning as the ring rolling step 84 provides sufficient de-scaling as will be discussed in greater detail below. The billet or slug 100 is then heated to an appropriate temperature for the deformation operations illustrated in FIG. 4. It has been found that, due to the greatly minimized heat loss of the workpiece experienced in the present practice as opposed to the process illustrated in FIG. 3, that heating of a billet to an appropriate temperature in the range of 2000° F. to 2300° F. is sufficient. It has also been found that for near net forgings of many of the alloys listed above, such as for example, AISA 8620A and 9310A, the normalizing heat treatment of

5  
10  
15

step 88 is not required. Experience has shown that the process illustrated in FIG. 4, for certain of the alloys listed above, provides good machinability of the precision near net forgings as the microstructure is a polygonal ferrite and pearlite equiaxed grain with no or only a minimum of, undesirable Widmanstatten structure. The grain size is generally fine (i.e. less than g.s. number 7 to 8 on the ASTM scale). Further, in view of the inherent de-scaling feature of the ring rolling process, heating of the billets for the precision forging of near net forging need not be in a controlled atmosphere.

The heated billet 100 is then forged into a trimmed ring rolling preform 102 having a generally toroidal shape in step 82. The details of forging the ring rolling preform symbolically illustrated by step 82 are illustrated in greater detail by reference to FIGS. 5, 6, 7 and 8, and will be discussed in greater detail below.

In step 84, the ring rolling preform 102 is ring rolled into a generally rectangular cross-sectional wall forging blank ring 104. The ring rolled forging blank ring 104 is then forged into a near net ring gear forging 106 in step 86.

An enlarged view of the details of the near net ring gear forging 106 may be seen by reference to FIG. 10. As will be discussed below, the height 108, wall thickness 110, inner diameter 112 and outer diameter 114 of the rolled forging blank ring 104 are required to be of specific relationships relative to the near net ring gear forging 106. The dimensions of the rolled forging blank 104 will also determine at least in part, the dimensions of the ring rolling preform 102.

The ring rolling process schematically illustrated at step 84 is well known in the prior art and may be appreciated by reference to FIG. 9. Briefly, the ring rolling preform 102 is placed over a rotatable mandrel 116 having an outer diameter slightly less than the inner diameter 118 of the preform. A relatively larger diameter king roll 118 will contact the outer diameter surface of the workpiece and will be rotatable driven to frictionally rotate the workpiece between the mandrel and the king roll. Either the king roll or the mandrel is then urged to move radially toward the other of the rolls to squeeze the workpiece therebetween. Ring rolling is relatively well known in the prior art and may be seen by reference to above-mentioned U.S. Pat. Nos. 4,084,419; 3,382,693; 3,230,370; 1,991,486 and 1,971,027 and by reference to Metals Handbook, 8th edition, volume 5, American Society for Metals, pages 106 and 107 "Ring Rolling".

Two inherent features of the ring rolling process are important to consider. During the ring rolling process the height 120 of the preform will not be substantially increased, and thus the height 120 of the preform will equal the height 108 of the rolled forging blank ring 104. The ring rolling process inherently will de-scale the workpiece eliminating the necessity for a separate de-scaling bustling operation and also the preform 102 and rolled ring 104 present a relatively small surface area in contact with the tooling and thus the ring rolling process represents a relatively minimal heat loss. The deformation heat generated may actually increase the temperature of the workpiece, allowing subsequent forging of a near net ring gear forging at the desired forging.

FIG. 4A illustrates the post metal deformation operations portion of the present invention. As stated above, certain alloys may require a normalizing heat treatment similar to that defined above for step 58 of the prior art

50  
30  
35  
40  
45

process. Many of the alloy steels utilized in the present invention will not require such a normalizing heat treatment of the near net gear forging 106.

Referring to FIG. 10, the near net gear forging 106 produced by the precision forging step 86 to the present invention is illustrated. In the illustration of FIG. 10, that portion of the near net forging located outwardly of the dotted lines will require removal to produce the final ring gear 14.

The near net forging 106 is semi-finish machined to drill the bolt circle bores 28 in the mounting flange 76, the mounting bore 28 and the backface 122. Drilling of the bolt circle bores is identical to step 62 of the prior art method while semi-finish machining of the mounting bore 28 and backface 122 is required to provide locating surfaces for further machining. During the semi-finish machining operation 90, some machining may also be required at the face angle and/or toe bore, depending upon the quality of the near net forging 106. The semi-finish machining workpiece is then subject to a carburizing heat treatment 92 substantially identical to step 68 described in connection with the prior art process.

After the carburizing heat treatment of step 92, the bolt circle bores 30 and mounting bore 28 are finish machine in step 94.

The process is then completed by finish grinding of the root and flanks of the gear tooth profiles in step 96. As the grinding of the final tooth profiles occurs after the carburizing heat treatment, a preferred method of grinding is by cubic boron nitride ("CBN") grinding which provides a suitably economical form of grinding carburized metallic surfaces. It is a highly desirable feature of the present invention that the final gear teeth profiles are provided after the final heat treatment operation and thus the ground tooth profile surfaces will not be subject to any heat treatment related distortion. Accordingly, assuming a pinion gear produced by a similar process, the ring gear and pinion gear lapping operations and maintenance of a lapped ring gear pinion gear gear set as a matched set is not required.

As indicated above, the method of the present invention, as symbolically illustrated in FIGS. 4 and 4A, provides substantial material and related energy and handling savings as compared to the prior art method as illustrated in FIGS. 3 and 3A. By way of example, and of comparing the two processes to provide a substantially identical part (Eaton Corporation, Axle and Brake Division, Part. No. 86374) the final product, ring gear 14, has a weight of approximately 49.75 pounds. The billet 32 utilized in the prior art process has a weight of approximately 103 pounds compared to the approximately 70 pound billet weight for billet 100 utilized in the process of the present invention. This does, of course, represent a material saving in excess of thirty percent (30%). Also, the weight of the untrimmed gear blank 52 will equal about 100 to 102 pound (i.e. billet weight less weight of removed scale) as compared to the approximately 64 pound weight of the near net ring gear forging 106. Accordingly, it may be seen that a substantially lower capacity press may be utilized by the present invention which will substantially increase the usable life of the forging tooling. Further, by utilizing a ring shaped forging blank 104, a flashless or substantially flashless near net forging die may be utilized. By way of further comparison, the trimmed gear blank 56 produced by the prior art invention will have a weight of approximately 78.5 pounds compared to the approximately 64 pound weight of the near net forging 106 of

the present invention giving an indication of the amount of metal of be removed in the rough cut and finish cut tooth cutting steps of the prior art method. Similar material savings, and related savings, on a percentage basis, have been demonstrated on both larger and smaller size heavy-duty drive axles ring gears produced by the method of the present invention.

In addition to material savings, the total process energy requirements, comprising the sum of: energy required for billet preparation, energy required for billet heating, forging energy, energy required for heat treatment after forging for proper machinability, the energy required for carburizing heat treatment, the energy required for post carburizing operations (lapping) and the energy required for machining, is at a minimal, or near minimal, level.

It is also noted that many of the gear-sets produced by the prior art methods require a shot peening or other tensile stress relief treatment after the carburizing heat treatment 68 to relieve the undesirable tensile stress in the carburized work pieces. In the present invention, shot peening or other tensile stress relief is not required as grinding, especially CBN grinding, tends to relieve tensile, and to induce desirable compressive, stress in the workpiece surfaces.

Referring to FIGS. 4 and 10, certain dimensional relationships of the roll forging blank ring 104 relative to the dimensions of the precision forged near net ring gear forging 106 must be maintained for optimal utilization of the process of the present invention. It has been found, that to achieve satisfactory fill of the precision forging die and to produce a satisfactory near net ring gear forging 106, that the height 108 of the rolled forging blank ring 104 must be in the range of one (1) to four (4), preferably, one and one-half (1½) to two and one-half (2½), times as great as the wall thickness 110 of the forging blank ring 104. Further, to properly locate in the precision forging die, the inner diameter 112 of the forging blank 104 must be substantially equal to the toe bore 124 (also referred to as the pot diameter of the die) and the outer diameter 114 of the rolled forging blank ring 104 must be less than the outside diameter 126 of the near net ring gear forging 106.

As is known in the prior art, the grain flow characteristics of gear teeth formed by metal deformation, such as by forging, are more desirable than the grain flow characteristics of teeth formed by a metal cutting operation and are thus of superior performance as to bending fatigue and the like. It is believed that the desirable grain flow of gears produced by the method of the present invention is due mostly to the forming of teeth by metal deformation, however, it is also believed that this tendency is enhanced by the utilization of a ring rolled gear forging blank. Grain flow developed in the gear teeth by forging to shape improves both the impact and fatigue properties over gears produced by machining the teeth from a solid blank such as blank 56.

The precision forging process by which the near net ring gear forgings 106 are produced involves a flashless or substantially flashless forging die and thus the volume of the ring rolled forging blank 104 must be very carefully controlled. The ring rolling equipment can be utilized over a wide range of preforms to be rolled into forging blanks as the height 120 of the preform will determine the height 108 of the blank 104 and thus by controlling the separation between the mandrel 116 and king roll 118 the wall thickness 110 and diameter 114, can be varied as required. It is, however, extremely

desirable that the preform required for each near net gear forging 106 not be of an entirely unique shape and not require a unique die for the forging thereof.

Applicant's have discovered, that so long as the height 108 of the rolled ring 104, and thus the height 120 of the forged preform 102, is within the range of one (1) to four (4), preferably one and one-half (1½) to two and one-half (2½), times the wall thickness 110 of the rolled ring, a very satisfactory precision forging operation can be obtained. Based upon this allowance, and applicant's discovery of a unique preform forging die cavity providing acceptable preforms of substantially toroidal shape provided the volume of the preform is within the range of one hundred percent (100%) to eight percent (80%) of the theoretical maximum toroidal volume of the die, applicant has been able to forge a family of different weight preforms utilizing the same die.

The process of the present invention is more fully illustrated referring to FIG. 5 which illustrates the further details of steps 80 and 82 of the process of the present invention, FIG. 6 which illustrates the unique die utilized therewith, and FIGS. 7 and 8 which illustrate the die as filled to one hundred percent (100%) and eight percent (80%), respectively, of the theoretical volume thereof.

The shape of the trimmed ring rolling preform 102 is preferably substantially toroidal defining a substantially circular cross-section along any radius thereof. The substantially circular cross-section is important and highly desirable as the ring rolling process tends to create a ring having substantially rectangular cross-sectional walls and during this ring rolling process substantially round surfaces of the workpiece will tend to prevent the formation of fish-tail and material from being folded over, either of which would create a defect in the near net forging as is known in the art. Repeating, the generally annular cross-section of a generally toroidal preform minimizes the likelihood of defects as the ring rolling process tends to square up the surfaces, and the rounded surfaces are less likely to have any folded defects or over portions.

Referring to FIG. 5, in step 80 of the process of the present invention, the round or round cornered square billet 100; is heated as described above, and is then upset into a pancake shaped billet 130 as seen in step 82A. In step 82B, the pancake shaped billet 130 is forged into a untrimmed preform 132 comprising a generally toroidal or ring-shaped portion 134 and a center or slug portion 136, by using the unique preform forging die 138 illustrated in FIGS. 6, 7 and 8. In step 82C the center slug is trimmed from the untrimmed preform 132 to provide the forged preform 102 for the ring rolling process.

Preform forging die 138 comprises upper and lower portions 140 and 142 that mate together at a parting line 144 to define a die cavity 146 therebetween. Die cavity 146 includes a radially inward generally disc shape portion 148, a generally toroidal shaped portion 150 extending radially outwardly from the disc shape portion 148, and an annular generally triangular shaped overflow portion 152 extending radially outwardly from the generally toroidal shape portion 150 and defined by generally flat surfaces 154 extending radially outwardly and towards the parting line from a point tangent to the generally toroidal shape portion 150 and defining an included angle 156 therebetween. Included angle 156 is in the range of 75° to 105°. The radially outward boundary of the generally toroidal portion 150 is indicated by the dotted line 158 in FIGS. 6-8.

The theoretical volume of cavity 146 of preform forging die 138 is the volume of portions 150 and 148. The theoretical volume of the toroidal portion 150 of cavity 146 is defined by the volume of portions 150 and 148 minus the volume of portion 148 which will remain substantially constant. Applicant's have discovered that toroidal shaped preforms having a volume of material which will fill the toroidal shaped cavity 150 of die 138 in the range of eight percent (80%) (see FIG. 8) to one hundred percent (100%) (see FIG. 7) of the theoretical volume of cavity 150 will provide preforms having a cross-sectional shape sufficiently circular to allow ring rolled into rectangular wall ring shaped forging blanks without defects. This is due to the shape of the die cavities 150 and 152 which tend to force the billet material into a generally annular cross-section ring having relatively smooth circular surfaces and a height 120 equal to the height of the cavity 150. Of course, the disc shaped portion 148 of cavity 146 will have a diameter 112 equal to the inner diameter 112 of the ring rolling preform which is slightly greater than the outer diameter of the ring rolling mandrel 116. It is also noted that for proper material flow, the height 162 of the disc shaped portion 148 should be approximately ten percent (10%) of the diameter 112 thereof. Should the variety of ring gear preforms 106 to be manufactured by the method of the present invention require more than one preform die 138, the diameter 112 and thickness 162 of the disc shaped portion 148 will remain substantially constant for all of the dies required.

Accordingly, to determine if a ring rolling preform 102 to be first rolled into a ring and then precision forged into a near net ring gear forging 106 of given outer diameter 126, tow bore 124 and volume can be forged in a given preform die 138 having a toroidal cavity portion 150 of known theoretical volume and known height 120 (or circular cross-section diameter) the following criteria must be satisfied: the volume of the near net ring gear forging 106 must be not more than one hundred percent (100%) and no less than eighty percent (80%), preferably no less than eighty five percent (85%) of the theoretical volume of the toroidal cavity portion 150; and, a generally rectangular forging blank 104 of a volume equal to the volume of the near net forging 106 and of a height 108 equal to the height 120 of the cavity portion 150 and an inner diameter 112 generally equal to the toe bore 124 of the forging must be providable with an outer diameter 114 less than the outer diameter 126 of the forging and of a wall thickness 110 having a relationship to the height 108 such that the height is no less than one times the thickness and no greater than four, times the thickness (preferably the ratio will be in the range of 1.5 to 2.5) of the ring wall.

If the above criteria are met, a preform may be forged in the given die 138 which will provide a satisfactory ring shaped forging blank upon ring rolling thereof. By establishing this criteria and ranges, the necessity for providing a plurality of preform forging dies is substantially reduced without detracting from the quality of the precision formed near net gear forgings. The shape of the die cavity 146, including especially the toroidal portions and the generally flat sided overflow portions which will tend to cause material to move radially inwardly is important to the present invention. As may be seen from the above, the process of the present invention provides a new and highly desirable method for the production of ring gears for heavy-duty drive axles and in particular, for the forging of ring rolling preforms to

be ring rolled into ring shaped forging blanks for precision forging to near net ring gear forgings of given dimension.

The above description of the preferred embodiment of the present invention is provided for illustrative purposes only and it is understood that the present invention is susceptible to modification, variation or change without departing from the spirit and the scope of the invention as hereinafter claimed.

I claim:

1. A method for forging a series of ring rolling preforms, each preform of said series to be ring rolled into a ring shaped forging blank for precision forging into a near net ring gear forging of known outside diameter, toe diameter and total volume, at least one of said outside diameter, toe diameter and total volume of the near net ring gear forging to be produced by each member of said series of preforms being different than the outside diameter, toe diameter and total volume of the near net ring gear forging to be produced by the other members of said series of ring rolling preforms, said method comprising:

providing a preform forging die having a die cavity comprising a substantially toroidal shaped portion of given volume and of given cross-sectional interior diameter, a disc shaped portion extending radially inwardly from said generally toroidal shaped portion and an overflow portion extending radially outwardly from said generally toroidal shaped portion, said overflow portion in cross-section being generally triangular shaped and defined by flat surfaces extending from said toroidal shaped portion radially outwardly and tangentially toward the parting surface of said die to define an included angle therebetween; and

forging preforms utilizing said preform forging die if the volume of the near net ring gear forging to be produced therefrom is in the range of eighty percent (80%) to one hundred percent (100%) of the volume of said toroidal cavity portion.

2. The method of claim 1 wherein said preforms are forged utilizing said preform forging die only if, given a known material to be forged, a ring having a generally rectangular cross-sectional wall with a height equal to the interior diameter of said die cavity toroidal shaped portion can be provided having an outer diameter less than said outside diameter, an inner diameter substan-

tially equal to said toe diameter and a radial wall thickness in the range of 1:1 to 1:4 of the ring height.

3. The method of claim 2 wherein said range of rectangular ring wall thickness to wall height is in the range of 1:1.5 to 1:2.5.

4. The method of claim 1 wherein the total volume of said near net ring gear forging must be at least eighty five percent (85%) of the volume of said toroidal section of said cavity.

5. The method of claim 2 wherein the total volume of said near net ring gear forging must be at least eighty five percent (85%) of the volume of said toroidal section of said cavity.

6. The method of claim 3 wherein the total volume of said near net ring gear forging must be at least eighty five percent (85%) of the volume of said toroidal section of said cavity.

7. The method of claim 1 wherein included angle is in the range of 70° to 110°.

8. The method of claim 1 wherein said included angle is about 90°.

9. A forging die for forging ring rolling preforms of generally toroidal shaped with the center slugs trimmed therefrom, said die comprising an upper and lower die member matable at a parting line to define a die cavity therebetween said die cavity comprising a generally toroidal shaped portion, a generally disc shaped portion extending radially inwardly from said toroidal shaped portion and an overflow portion extending radially outwardly from said toroidal shaped portion, said overflow portion of generally triangular shape in cross-section and defined by a pair of flat surfaces converging at said parting line, said generally flat surfaces extending tangentially from said toroidal shaped portion and extending radially outwardly and toward said parting line to define an included angle therebetween, said included angle in the range of 60° to 120°.

10. The preform forging die of claim 9 wherein said included angle is in the range of 70° to 110°.

11. The preform forging die of claim 9 wherein said included angle is about 90°.

12. The preform forging die of claim 9 wherein said disc shaped portion is of a height approximately ten percent (10%) of the diameter thereof.

13. The preform forging die of claim 11 wherein said disc shaped portion is of a height approximately ten percent (10%) of the diameter thereof.

\* \* \* \* \*